

## UNITED STATES PATENT OFFICE

WALTER TAUSSIG, OF FRANKFORT-ON-THE-MAIN, GERMANY, ASSIGNOR TO DURAND & HUGUENIN, OF BASEL, SWITZERLAND, A CORPORATION OF SWITZERLAND

PROCESS FOR PRINTING WOOL WITH ESTER SALTS OF LEUCO COMPOUNDS OF VAT DYESTUFFS

No Drawing. Application filed October 12, 1928, Serial No. 312,209, and in Germany October 13, 1927.

My invention relates to a process for printing wool with ester salts of leuco-compounds of vat dyestuffs. These ester salts well known in the practice are applied in a wide extent for printing cotton and for dyeing wool. But for printing wool they could not be used hitherto because there was not known a suitable oxidizing agent which develops sufficiently the dyeing of the ester salt but does not stain the nonprinted part of the woolen fabric.

I have now found that ester salts of leuco-compounds of vat dyestuffs when printed on wool are developed in an excellent fastness, without staining the white part of the woolen fabric, by means of solutions of persulfates mixed with strong acids as sulfuric or hydrochloric acid. A special advantage of my present process consists in the fact that the print pastes contain only a thickening agent besides the solution of ester salts of the leuco-compounds of vat dyestuffs.

Only when such ester salts of leuco-compounds of vat dyestuffs are applied which are too difficult to be reoxidized, some persulfate is advantageously admixed already to the printing color.

In order to further illustrate my invention the following examples are given, the parts being by weight and all temperatures in Centigrade degrees. But I wish to be understood that I am not limited to the particular conditions nor to the specific products mentioned therein.

*Example 1*

A woolen fabric is printed with a printing paste prepared as follows:

Sulfuric acid ester salt of the leuco-compound of:

|                                                                                      |      |      |      |      |
|--------------------------------------------------------------------------------------|------|------|------|------|
| 6.6'-diethoxy-thioindigo, parts                                                      | 70   |      |      |      |
| 5.7.6'-trichloro-indigo, parts                                                       |      | 50   |      |      |
| 5.7.5'.7'-tetrabromo-indigo, parts                                                   |      |      | 80   |      |
| The dyestuff prepared according to Example 1 of the German Patent No. 241,997, parts |      |      |      | 125  |
| Parts of water                                                                       | 330  | 350  | 320  | 275  |
| Parts of British gum 1:1                                                             | 600  | 600  | 600  | 600  |
| Parts                                                                                | 1000 | 1000 | 1000 | 1000 |

After having been printed and dried the goods are steamed for about half an hour in

the manner usual for printed wool and developed at 50-70° in a bath containing per liter 10-20 parts of potassium persulfate and 12-30 parts of hydrochloric acid 20° Bé. or the equivalent amount of sulfuric acid. Then they are rinsed, soaped as usually, rinsed again and dried.

*Example 2*

Woolen material is printed with the following print-paste:

Sulfuric acid ester salt of the leuco-compound of

|                                                 |      |     |
|-------------------------------------------------|------|-----|
| 4.4'-dichloro-6.6'-dimethyl - thioindigo, parts | 40   | 65  |
| Parts of water                                  |      | 340 |
| Parts of British gum 1:1                        |      | 600 |
| Parts of potassium persulfate                   |      | 20  |
| Parts                                           | 1000 | 70  |

The printed fabric is developed as described in Example 1.

*I claim:*

1. A process which comprises printing woolen fabrics with a printing paste containing a thickening agent and a solution of an ester-salt of a leuco compound of a vat dyestuff, drying and steaming the printed fabrics and treating them with a strong mineral acid in combination with a persulfate as oxidizing agent, this latter being admixed at any stage of the process and being incapable of staining the white parts of the woolen fabrics.

2. A process which comprises printing woolen fabrics with a printing paste containing a thickening agent and a solution of an ester salt of a leuco vat dyestuff, drying and steaming the printed fabrics and treating them with a solution containing a strong mineral acid and a persulfate as oxidizing agent incapable of staining the white parts of the woolen fabrics.

3. A process which comprises printing woolen fabrics with a printing paste containing a thickening agent and a solution of an ester salt of a leuco compound of a vat dyestuff, drying and steaming the printed fabrics and treating them with a solution containing

hydrochloric acid and a persulfate as oxidizing agent incapable of staining the white parts of the woolen fabrics.

4. A process which comprises printing  
5 woolen fabrics with a printing paste containing a thickening agent and a solution of an ester salt of a leuco compound of a vat dye-stuff, drying and steaming the printed fabrics and treating them with a solution containing  
10 per liter from 12 to 30 parts of hydrochloric acid 20° Bé. and from 10 to 20 parts of potassium persulfate, at a temperature of 50° to 70° C.

15 In testimony whereof, I affix my signature.  
**WALTER TAUSSIG.**

**20****25****30****35****40****45****50****55****60**